

## [54] METHOD OF RESTRICTING THE OXIDATION OF SPONGE IRON

[75] Inventors: **Wilhelm Thumm**, Frankfurt am Main; **Horst Nagel**, Bergen-Enkheim, both of Germany

[73] Assignees: **Metallgesellschaft Aktiengesellschaft**, Reuterweg, Germany; **The Steel Company of Canada, Ltd.**, Hamilton, Ontario, Canada

[22] Filed: Aug. 12, 1971

[21] Appl. No.: 171,109

## [30] Foreign Application Priority Data

Sept. 11, 1970 Germany ..... P 19 27 300.8

[52] U.S. Cl. .... 21/2.5, 75/0.5 R

[51] Int. Cl. .... C23f 11/02, C23f 9/02

[58] Field of Search ..... 21/2.5; 75/26, 0.5 R

## [56] References Cited

## UNITED STATES PATENTS

1,896,478 2/1933 Burns ..... 21/2.5 UX

|           |         |                       |           |
|-----------|---------|-----------------------|-----------|
| 2,156,357 | 5/1939  | Simpson .....         | 21/2.5 UX |
| 2,160,831 | 6/1939  | Colby et al.....      | 21/2.5 UX |
| 2,616,780 | 11/1952 | Atkinson et al. ....  | 21/2.5    |
| 2,677,669 | 5/1954  | Ahlberg.....          | 252/472   |
| 3,111,371 | 11/1963 | Bull.....             | 21/2.5    |
| 3,188,166 | 6/1965  | Dietz et al. ....     | 21/2.5    |
| 3,551,215 | 12/1970 | Claiborne et al. .... | 75/26 UX  |
| 3,562,780 | 2/1971  | Eisenberg.....        | 75/26     |

## FOREIGN PATENTS OR APPLICATIONS

649,735 1/1951 Great Britain..... 21/2.5

Primary Examiner—Barry S. Richman

Attorney—Karl F. Ross

## [57] ABSTRACT

The oxidation of sponge iron, as generally made by the direct reduction of an iron ore, is prevented or limited by circulating through the mass of sponge iron a gas stream containing air and/or nitrogen together with ammonia.

5 Claims, 1 Drawing Figure





Karl G. Ross  
Attorney

## METHOD OF RESTRICTING THE OXIDATION OF SPONGE IRON

### CROSS-REFERENCE TO RELATED APPLICATION

This application is related to the copending application Ser. No. 39,630, filed 22 May 1970 by us together with others, and entitled METHODS OF AND APPARATUS FOR RESTRICTING OXIDATION OF SPONGE IRON; the present application is commonly assigned with the earlier application.

### FIELD OF THE INVENTION

Our present invention relates to a method of preventing the reoxidation of sponge iron or of restricting such reoxidation and, more particularly, to a method of and an apparatus for limiting the oxidation of sponge iron in bulk.

### BACKGROUND OF THE INVENTION

Sponge iron is generally produced by the direct reduction of iron oxide, generally in the form of briquettes or pellets, to produce a mass of elemental iron of relatively high purity without a smelting process. The iron has a sponge structure, i.e. is highly porous or cellular, and thus has a high surface-area/weight or surface-area/volume ratio and thus is susceptible to reoxidation in the presence of atmospheric oxygen and, generally, atmospheric moisture. Various suggestions have been made as to how to avoid reoxidation of the sponge iron, such reoxidation having numerous disadvantages. Firstly, reoxidation may introduce a large proportion of oxygen into the metal structure and require special treatment during steel-making or other refining processes. Secondly, the oxidation process is exothermic and stored bulk sponge iron can show a spontaneous increase in temperature to 80° to 100° C or even to the point of ignition. Such temperature rises are especially disadvantageous when the sponge iron is stored in the hold of a ship because of thermal stress on the hull or otherwise endanger this conveyance.

Consequently, it has been suggested to coat the mass of sponge iron with an antioxidation or anticorrosion substance such as oil, paraffin or a synthetic resin. These systems have the obvious disadvantage that they apply other impurities to the iron, are expensive and may not provide adequate protection within the cellular body of the mass. Other methods have been suggested as well, but these have only been applied successfully to small quantities of sponge iron, i.e. bags or sacks thereof. Even techniques for storing the sponge iron under a nonoxidizing atmosphere have not proved to be fully satisfactory.

### OBJECTS OF THE INVENTION

It is the principal object of the present invention to provide an improved method of limiting the oxidation or reoxidation of sponge iron which is relatively inexpensive, effective and free from the disadvantages of earlier systems as described above.

It is another object of the invention to provide a system for reducing or restricting the oxidation of agglomerated sponge iron, preferably in bulk, during storage and transition.

Yet another object of the invention is to provide a method of and an apparatus for limiting oxidation of sponge iron in lump or agglomerated form which are relatively inexpensive and free from the indicated disadvantages.

Still another object of the invention is to provide a system for the purpose described that does not deposit impurities on the iron.

Yet a further object of the invention is to provide a method of restricting the reoxidation of sponge iron which advances the principles set forth in the commonly owned copending application Ser. No. 39,630, filed 22 May 1970.

### SUMMARY OF THE INVENTION

In the above-identified application, it has been pointed out that the reoxidation of sponge iron can be limited or restricted surprisingly, by passing a gas stream through the mass, in spite of the fact that the gas may include air or atmospheric oxygen. While one normally would expect that treatment of a sponge-iron mass with an oxygen-containing gas stream would promote oxidation rather than restrict it, the contrary is true apparently because the gas stream prevents static contact between ambient gases and the sponge iron and removes moisture from the vicinity of the interface. We have now found that the oxidation-limiting effect can be increased by incorporating in the gas stream contacted with the sponge iron between 1 and 160 g of ammonia per m<sup>3</sup> (standard temperature and pressure - STP) of the gas stream circulated through the sponge iron.

With respect to the concept of circulating a gas stream through the sponge iron to reduce the tendency toward reoxidation, the aforementioned application provides for the steps of piling the agglomerated or lump sponge iron in an enclosure having a series of gas nozzles in the bottom, and passing through the sponge-iron mass, a gas such as air, nitrogen nitrogen-enriched air. The rate at which the gas is passed through the mass, determines the rise in temperature thereof so that a rate can be selected to give virtually no rise in temperature or a rise only to the highest possible limit tolerable by the conveyance or storage facility and short of combustion. As pointed out in that application, it was found that the oxidation rate and resultant temperature rise are dependent upon the rate of gas flow, and also, that the moisture content of the gas is a major contributing factor to oxidation of the iron mass. A dehumidifier is provided to remove moisture present in the gas prior to its passage through the mass. The dehumidifier may drop the temperature of the gas and thus a heater may be provided to raise the temperature and, of course, increase the dewpoint. It is therefore important in accordance with the principles of that application to reduce the water-vapor partial pressure as low as possible. The aforementioned application also points out that it is advantageous to collect and recycle the gas, in which case a blower is provided in addition to the dehumidifier and heater while a lime filter can be used to remove any acid constituents which may have been picked up by the gas passing through the iron mass. Such acid constituents have a strong oxidizing action.

60  
65

As noted earlier, the present invention resides in the addition to the gas traversing the sponge-iron mass of ammonia ( $\text{NH}_3$ ), preferably when the sponge iron is a powder, the gas being otherwise constituted as described in the aforementioned application. The use of ammonia eliminates the need for separate neutralization of acid constituents and also is effective to reduce the oxidation of the sponge-iron still further.

The ammonia can be sprayed in a liquid state continuously or discontinuously in constant or variable quantity and may be applied to the sponge iron directly, may be mixed with the gas stream traversing the sponge-iron mass in the receptacle therefore, or may be mixed with the gas elsewhere along the recirculating path. According to the feature of the invention, the ammonia may be supplied to the oxidation-limiting gas stream by spraying it in liquid form directly from above onto the sponge iron. In this case and generally, we prefer to induce a downward flow of the gas (including the ammonia) through the sponge-iron mass.

According to still another feature, the ammonia is supplied such that 1 to 160  $\text{g/m}^3$  (STP) constitutes its concentration in the gaseous oxidation-limiting medium, the concentration preferably being 2 to 50  $\text{g/m}^3$  (STP). It has been found that best results are obtained with quantities and flow rates of ammonia-containing gas ranging between 1 and 15  $\text{m}^3$  (STP) per  $\text{m}^2$  of the cross-section of the sponge iron, per hour. The quantity is dependent upon the height of the sponge-iron mass and increases with increasing height. The ammonia-containing gas is totally or partially circulated through the sponge-iron mass to minimize ammonia loss and the water vapor partial pressure is reduced in a condenser or other water-removal device. It is of course possible simply to pass the ammonia-containing gas through the sponge-iron mass without recirculation. A slight warming of the ammonia-containing gas, especially when the latter has been subjected to water removal, is also desirable.

The supply of the ammonia to the gaseous medium or to the sponge iron can be controlled in any convenient manner although we prefer to sense the temperature of the sponge-iron mass or the gases effluent therefrom and to regulate the ammonia supply in accordance therewith. With a temperature increase, the ammonia content is increased and vice versa.

A significant advantage of the present system is that the reoxidation of the sponge iron is reduced even more than has been possible with the system described in the aforementioned application at relatively low cost so that for any given tolerance of reoxidation and any given mass of sponge iron, the ducts, blowers and valves may be dimensioned somewhat smaller.

We have found that at heights of 1 to 3 m of the sponge-iron pile, the total gas-flow rate should range between 5 and 40  $\text{m}^3$  (STP) / $\text{m}^2$ -hour, preferably 8 to 25  $\text{m}^3/\text{m}^2\text{-hour}$ . With stacks or piles having a height of 3 to 8 meters, the total gas-flow rate should be 10 to 80  $\text{m}^3/\text{m}^2\text{-hour}$ , preferably 20 to 50  $\text{m}^3/\text{m}^2\text{-hour}$ . With stacks of a height in excess of 8 m, the gas-flow rate should be 20 to 160  $\text{m}^3/\text{m}^2\text{-hour}$ , preferably 40 to 100  $\text{m}^3/\text{m}^2\text{-hour}$ . With sponge-iron pile heights above 8 m, the supply of ammonia-containing gas should be 7 to 15  $\text{m}^3/\text{m}^2\text{-hour}$ , while heights of 3 to 8 m call for ammonia-containing gas supply rates of 3 to 10  $\text{m}^3/\text{m}^2\text{-hour}$ , and

pile heights of 1 to 3 m require from 1 to 8  $\text{m}^3/\text{m}^2\text{-hour}$  (STP) of ammonia-containing gas.

#### DESCRIPTION OF THE DRAWING

The above and other objects, features and advantages of the present invention will become more readily apparent from the following description, reference being made to the accompanying drawing in which the sole FIGURE is a flow diagram of a system embodying the present invention.

#### SPECIFIC DESCRIPTION

In the drawing, we have shown a vessel 10 adapted to receive a charge 29 of sponge iron above a grate 11 having perforations 12 communicating with a wind box 13. A blower 15, connected by the inlet pipe 14 to the storage vessel 10, induces a downward flow of gas through the vessel and supplies the gas to a condenser 16 in which it is cooled to precipitate moisture and reduce the water-vapor partial pressure. The cool gas is returned at 17 via a heater 18 to the top of the vessel. The top of the vessel 19 and the bottom thereof may be removed for filling and discharging the sponge-iron mass respectively. Atmospheric air, nitrogen, or air enriched with nitrogen can be led into the system through a valve 21 and an inlet 20.

Liquid ammonia from a tank 25 is supplied via a valve 24 and a pipe 22 to a spray head 23 above the sponge iron. Thermocouples 27 and 28 are provided to regulate the valve 24 and control the flow of ammonia into the system via a control line 26. When recirculation of the ammonia-containing gas stream is not desired, a valve 31 can be opened to discharge the gas at the discharge side of the blower 15. The spray 30 of ammonia is here shown to be directed onto the top of the sponge iron.

#### SPECIFIC EXAMPLE

A cylindrical vessel having a diameter of 0.5 m and a height of 3 m is filled with 830 kg of fresh sponge iron. The sponge iron is traversed by 25  $\text{m}^3/\text{m}^2\text{-hour}$  (STP) of atmospheric air at a temperature of 30°C which is recirculated through the system. Ammonia is introduced into the recirculated gas stream to a concentration of 50 g per  $\text{m}^3$  (STP) and the gas flow is adjusted so that about 5  $\text{m}^3$  of ammonia-containing gas (STP) passes through the sponge iron per  $\text{m}^2$  of cross-section per hour. With slight modification of the ammonia concentration, it is possible to maintain the temperature of the sponge-iron content at 30°C, the gas effluent from the sponge iron being cooled to 20°C prior to reheating to remove moisture. There is no noticeable oxidation of the sponge iron with time after the initial slight oxidation over a period of 10 hours. Without the ammonia, oxidation appeared to continue for some time.

We claim:

1. A method of preventing oxidation of sponge iron, comprising the steps of piling and enclosing sponge iron to form a gas-permeable mass thereof and passing a gaseous mixture of ammonia with a gas selected from the group consisting of air, nitrogen-enriched air and nitrogen through said mass at a rate of from substantially 1 to 15  $\text{m}^3$  (STP) per  $\text{m}^2$  of cross-section of the

mass per hour, the concentration of the ammonia in said gaseous mixture being between 1 and 160 g/m<sup>3</sup> (STP), and further comprising the step of reducing the water-vapor partial pressure in said gaseous mixture prior to passing said gaseous mixture through said mass.

2. The method defined in claim 1 wherein said concentration is 2 to 50 g per m<sup>3</sup> (STP).

3. The method defined in claim 1 wherein the am-

monia is introduced into the gaseous mixture by spraying liquid ammonia onto said sponge-iron mass.

4. The method defined in claim 1 wherein the gaseous mixture is recirculated through said mass.

5. The method defined in claim 4, further comprising the step of heating said gaseous mixture prior to passage thereof through said mass.

\* \* \* \* \*

10

15

20

25

30

35

40

45

50

55

60

65

UNITED STATES PATENT OFFICE  
CERTIFICATE OF CORRECTION

Patent No. 3,723,059 Dated 27 March 1973

Inventor(s) Wilhelm THUMM et al

It is certified that error appears in the above-identified patent  
and that said Letters Patent are hereby corrected as shown below:

In the heading, line "30, for the German appli-  
cation serial number read -- P 20 45 022.0 -- .

Signed and sealed this 28th day of August 1973.

(SEAL)

Attest:

EDWARD M. FLETCHER, JR.  
Attesting Officer

RENE D. TEGTMEYER  
Acting Commissioner of Patents